# EUROPEAN PATENT SPECIFICATION

(11) **EP 1 840 487 B1**
(45) Date of publication and mention of the grant of the patent: **30.10.2013**
(21) Application number: 06112083.8
(22) Date of filing: 31.03.2006
(51) Int. Cl.: F25B 41/06, B23P 15/00, C22C 21/00, C22F 1/04, B21C 1/22, B21C 23/08

(54) **Endless capillary tubes in aluminium alloy and lamination valves comprising aluminium alloy capillary tubes**
Endloskapillarrohr in Aluminiumlegierung und Drosselventil mit diesen Endloskapillarrohr in Aluminiumlegierung
Capillaire en alliage d'aluminium et soupape d'étranglement comprenant ce capillaire en alliage d'aluminium

(43) Date of publication of application: 03.10.2007
(73) Proprietor: ARO TUBI TRAFILERIE S.P.A., 20122 Milano (IT); C.R. S.R.L., 25080 Moniga Del Garda (IT)
(72) Inventor: FOGARI, Riccardo, 25100, BRESCIA (IT); GUGLIELMINI, Alessandro, 20151, MILANO (IT)
(74) Representative: Weisgerber, Stefan

(56) References cited:
- WO-A-02/055256
- WO-A-03/106901
- DE-A1- 1 807 516
- FR-A- 2 836 542
- GB-A- 2 272 506
- GB-A- 2 376 513
- GB-A- 2 418 478
- JP-A- 6 278 243
- US-A- 2 687 626
- US-A- 3 923 557
- US-A- 4 408 467
- US-A1- 2001 007 720
- US-A1- 2001 025 676

## Description

### FIELD OF THE INVENTION.

The present invention relates to new "endless" capillary tubes, used preferably in the production of lamination valves.

### BACKGROUND ART.

In cooling circuits mounted on electrical household appliances, it is common practise to use capillary tubes as lamination valves, adapted to regulate the thermodynamic cycle of the circuit. In these capillary tubes, the length and the internal diameter basically determine the pressure drop of the cooling means used in the circuit. Therefore in the aforesaid valves the so-called flow rate of the capillary tubes employed, constitutes, together with the choice of fluid used, the key factor for the dimensioning and project design of the whole cooling system.

GB-A-2376513 discloses an example of heat transfer element for use within a refrigeration system wherein the heat transfer tubing portion is made of aluminium, in particular Al 3103.

For this reason it is important that this flow rate is maintained within very strict tolerance levels. The term "flow rate" refers to the volume of fluid (generally nitrogen or dry air is used as measuring fluid or gas) that passes through the section of the capillary tube during a unit of time at a determined inlet pressure. The flow rate is conventionally measured in litres per minute. In industrial practise the flow rate of a capillary tube is measured according to UNI EN 12450 standards. In fact, specific instruments are available on the market designed for this purpose. Preferably, in order to measure the flow rate, the gas is sent into the capillary tube at a pressure between 0.5 and 20 bar, more preferably between 4 and 15 bar. Even more preferably, the measuring gas pressure ranges between 5 and 10 bar.

Given that in industrial production of these valves destined for use in household appliances mass produced in vast quantities, it would be far too laborious to individually adjust the internal volume of every single capillary tube used in valve construction, by means of (1) individual measurement, using the aforesaid fluid mechanics, of its flow rate and (2) successive adjustment of its length, the household appliance industry requests capillary tubes of its suppliers that are extremely long (practically "endless"), whose internal volume (defined, as stated previously, through the "flow rate") is strictly proportional with the length, in other words, whose interior must be completely clean of all production residue and must be characterized by a constant diameter . This is in order to avoid individual interventions of the type (1) and/or (2) on each single capillary tube employed in the valve, and to ensure that it is possible to obtain the exact flow rate as designed by simply dividing the endless capillary tube supplied, in pieces of a suitable length, destined for use as lamination valves.

At present, the capillary tubes destined for the aims specified herein, are produced as "endless" tubes wound in rolls (so-called wound coils) and obtained through continuous machining comprising a succession of cold-drawning operations with a floating chuck on roughly semi-machined blanks obtained through extrusion. To guarantee the constant level of the capillary tube flow rate, it is essential that the internal diameter be constant, and it is thus important that materials in use possess well-defined chemical, physical and mechanical characteristics. Other important characteristics that are required and that cannot be modified because these are dictated by the preferred use are the resistance of the employed material to corrosion, as well as its compatibility with the fluids and other materials used in the cooling circuit. As the reader will become aware, the complexity of the problems described herein originate above all in the enormous difference between the size of the various dimensions of the "endless" tubes described herein, given that the length can reach as much as 5 kilometres in some cases, while the internal diameter does not exceed a few millimetres. For this reason, to guarantee the constant levels necessary for the flow rate along the total length of the endless capillary tube has required considerable productive effort in the past, both as far as materials are concerned, as well as the tools used.

For these reasons, the only material that has been considered actually usable (and is actually used) in the production of wound coil "endless" capillary tubes, able to provide very high constancy levels for the flow rate, is copper and its alloys.

This results in the fact that all the lamination valves mounted in cooling circuits in household appliances in common mass-produced industrial production are in copper or copper alloy. Therefore, the machinery used in this technical field is optimised for machining this metal. At present, the exclusive use of copper in this technical field ties the actual market price for these common lamination valves for household appliance cooling circuits, very closely to the price of the raw materials. The result is that, given increasing industrialisation in emerging countries under development, and given the increased needs for raw materials, the price of copper (LME) has increased in the last ten years alone, from 2610 US$ per ton in 1996 to over 5000 US$ per ton (02/2006). Given the large number of pieces obtainable with machinery available, this price has a considerable effect on that of the lamination valves obtained from copper and its alloys. In the immediate future, and in any case, in the medium term, this situation will become far worse because of the fact that in these same emerging countries under development, and above all in those even less developed countries, at the same time, and as an indicator of a constant improvement in the lifestyle quality, there is an increase in the demand for household appliances for immediate necessity (such as refrigerators), on condition that the price is not too high.

This has led to the need for obtaining capillary tubes with a constant flow rate, in the form of endless tubes, preferably wound in rolls or coils, preferably to be used to obtain lamination valves for household appliance cooling circuits from an alternative material, also less costly and less valuable than copper. Therefore there is a definite need for the provision of new lamination valves available for household appliance cooling circuits, in which the capillary tube, while providing the same performance level, is composed of a more economical alternative material. Moreover, it would be particularly advantageous if the said new lamination valves comprise a capillary tube composed of a material that is more resistant to corrosion and particularly suitable for use in the context of cooling circuits.

For this reason it is necessary that a material be found for the aforesaid uses, as an alternative to copper and its alloys, a material that is less valuable but just as easily machined.

### SUMMARY.

This problem is solved by the Applicants of the present invention, as disclosed in claims 1-10 by providing an endless capillary tube in aluminium alloy of the type having an internal diameter between the range 0.2 - 4.5 mm and a length within the range 100-10000 mm characterised in that the flow rate of two segments of the capillary tube having a length of 2500 mm cut from two positions taken at random from the endless capillary tube do not vary more than ±6%. Therefore, the endless capillary tube according to the present invention can be used for example, without any further adjustment to the single capillary tubes obtained from it to form the lamination valves for household appliances.

The present invention also provides a method for the production of endless capillary tubes according to claim 4 in an aluminium alloy, particularly suitable for the aforesaid aims, since it is able to be used on existing machines without the need for any modifications.

### DETAILED DESCRIPTION OF THE INVENTION.

In particular, in order to provide a solution to the aforesaid technical problem, in other words, in searching for an alternative material, preferably less costly, but just as easily used for the production of endless capillary tubes with a constant flow rate in rolls or wound coils, the inventors of the present application have surprisingly discovered that it is possible to use aluminium alloy for this purpose. Certain aluminium alloys are particularly preferable.

Within the context of the present invention, the term "capillary tube" refers to a tube whose internal diameter is very small, in particular, 4.5mm or less. Preferably, the internal diameter is such that the behaviour of a fluid in the tube interior, in particular a fluid commonly used in household appliance cooling circuits, is controlled by the so-called physical principle of capillarity. Therefore, more preferably, the capillary tubes of the present invention are characterised by an internal diameter less than 3mm, even more preferably less than 1.0mm. More preferred capillary tubes have an internal diameter less than 0.7mm. The minimum diameter of the capillary tubes according to the present invention is 0.2mm, preferably 0.3mm, more preferably 0.4mm, and most preferably 0.5mm.

Therefore, the capillary tubes of the present invention have an internal diameter 4,5mm or less, preferably less than 3mm, more preferably less than 1 mm, even more preferably less than 0.7 mm.

The capillary tubes of the present invention have an internal diameter that ranges between 4,5mm and 0.2 mm, preferably between less than 3mm and 0.2mm, more preferably between less than 1 mm and 0.2mm, even more preferably between less than 0.7 mm and 0.2mm.

Preferably the capillary tubes of the present invention have an internal diameter between 4.5mm and 0.3 mm, preferably between less than 3mm and 0.3mm, more preferably between less than 1 mm and 0.3mm, even more preferably between less than 0.7 mm and 0.3mm.

More preferably the capillary tubes of the present invention have an internal diameter that ranges between 4.5mm and 0.4 mm, preferably between less than 3mm and 0.4mm, more preferably between less than 1 mm and 0.4mm, even more preferably between less than 0.7 mm and 0.4mm.

Most preferable among the capillary tubes of the present invention have an internal diameter ranging between 4.5mm and 0.5 mm, preferably between less than 3mm and 0.5mm, more preferably between less than 1 mm and 0.5mm, even more preferably between less than 0.7 mm and 0.5mm.

Within the context of the present invention the term "endless" capillary tube refers to a seamless capillary tube obtained by means of continuous production. Said "endless" capillary tube is at least 100 metres long, preferably at least 500 metres long, even preferably at least 1000 metres long. Preferably, the endless capillary tube is wound to form rolls or wound coils.

The endless capillary tubes in aluminium alloy of the present invention are characterised by a very strict proportionality between flow rate and length. In particular, the flow rates of two segments of capillary tube having a length of 2500mm cut from two positions taken at random from the endless tube, do not vary by more than ±6%, preferably ± 3%, even more preferably ± 2% and most preferably ± 1%.

Therefore, it is possible to obtain from the aforesaid endless capillary tube in aluminium alloy by means of simple division, single capillary tubes having a predetermined length, ranging between 100mm and 10 000mm, preferably between 500mm and 5000mm, more preferably between 1000mm and 3000mm, providing a consequential flow rate, preferably destined to obtain lamination valves for household appliances. The proportionality between length and flow rate of said single capillary tubes is such that if the capillary tubes according to the present invention are in turn, also cut in half, the flow rates of the resulting two halves will not differ by more than ± 6%, preferably ±3%, even more preferably 2%, and most preferably 1%.

The production of endless capillary tubes in aluminium alloy according to the present invention is obtained using common processes already in practise in the sector for the production of traditional endless capillary tubes in a known copper alloy.

For example the production of endless capillary tubes in aluminium alloy occurs according to a process comprising the following steps:
- Hot extrusion of a rough blank;
- Successive stages of cold drawing, the number of stages depending on the envisaged machining cycle; the external diameter and the tube thickness are reduced with each extrusion stage until the final measure is obtained;
- Winding to form wound coils;
- Washing of the internal surface to eliminate machining residue (lubricants, etc.);
- heat treatment aimed at modifying the mechanical characteristics of the capillary tube increasing the ductility.

As stated previously, a fundamental characteristic of the endless capillary tubes as well as their segments as defined previously, and above all of single capillary tubes (obtained from endless tubes) described herein -according to the present invention and unlike traditional tubes already widely used, is the fact that for the first time tubes are obtained from an aluminium alloy.

When the endless capillary tube in aluminium alloy according to the present invention, divided to form the single particular capillary tubes used for lamination valves and placed in comparison with similar copper capillary tubes, the aluminium tube is able to guarantee:
- At least equivalent performance, preferably even better, in terms of flow rate constancy;
- Mechanical characteristics that permit handling and assembling of the component in cooling circuits without any particular restrictions;
- Strong resistance to corrosion (over 500 hours in ASTM G85-98 A3).

Research performed by the inventors of the present Application has also demonstrated that it is possible to obtain on machinery commonly destined for the production of traditional endless capillary tubes in copper o copper alloy, without the need for any modification-capillary tubes in an aluminium alloy, consisting of: Si: 0.15% in weight max; Fe: 0.25% in weight max.; Cu: 0.10% in weight max.; Mn: 0.90-1,10% in weight; Mg: 0.06% in weight max.; Cr:0.06% in weight max.; Zn: 0.10% in weight max.; Ti: 0.06 % in weight max.; the remainder being aluminium and inevitable impurities.

A preferred aluminium alloy consists of: Si: 0.10% in weight max.; Fe: 0.20% in weight max.; Cu: 0.10% in weight max.; Mn: 0.90 -1,10% in weight; Mg: 0.03% in weight max.; Cr: 0.03% in weight max.; Zn: 0.07% in weight max.; Ti: 0.03% in weight max.; the remainder being aluminium and inevitable impurities.

Particularly preferred is an aluminium alloy consisting of: Si: 0.10% in weight max.; Fe: 0.15% in weight max.; Cu: 0.10% in weight max.; Mn: 1.00 - 1.10% in weight; Mg: 0.03% in weight max.; Cr: 0.03% in weight max.; Zn: 0.07% in weight max.; Ti: 0.03% in weight max.; the remainder being aluminium and inevitable impurities.

From the experiments performed by the inventors of the present Application it has appeared that the combination of the elements described above, (exemplified by the three alloys described) can guarantee the workability levels necessary to obtain the "endless" tubes described herein, and that they are particularly suited to achieve the aims of the present invention.

As stated previously, the aluminium alloy identified above permit the production of endless capillary tubes of the present invention, using the same processes used to produce endless capillary tubes in copper, without the need for any modifications.

The aluminium alloy according to claim 1 permits continuous production without the forming of faults or rupture during the working.

In particular, by using the aluminium alloy according to claim 1, the machine tools traditionally optimised for the production of copper capillary tubes can be used to total benefit without the need for modification.

This is because the use of an aluminium alloy that belongs to the general class 3103 (in other words aluminium alloy composed of Si: 0.50% in weight max.; Fe: 0.70% in weight max.; Cu: 0.05% - 0.10% in weight; Mn: 0.90 - 1.50% in weight; Mg: 0.30% in weight max.; Cr: 0.10% in weight max.; Zn: 0.20% in weight max.; Ti: absent, the remainder being aluminium and inevitable impurities), as defined by UNI EN 9003/3 standards, is not sufficient to guarantee material workability of a level that permits continuous production of capillary tubes with homogeneous quality with the current technology available. In fact, within this class alloys exist with similar compositions, but with different performance levels in terms of mechanical characteristics, even up to a level of 25 %: this fact makes it impossible to obtain constant production (continuous and with homogeneous quality) using machinery currently available.

For example, with an alloy of the identified composition but with a magnesium content equal to 0.30% (outside the object of the present invention but within class 3103), a material is obtained that has low workability levels and consequential frequent rupture of the capillary tubes.

In addition, the reduction of the maximum Fe content from 0.70 % (alloy 3103) to 0.25 % provides an improvement in productivity and the surface quality of the product because of a lesser quantity of precipitates with abrasive action.

For example, an alloy with the identified composition but with an Fe content equal to 0.40 % (outside the specific object of the present invention but within class 3103) produces roughness on the extruded tube equal to 2,5 µm (Ra) compared to 1 µm (Ra) of the alloy object of the invention. During the successive operations, the alloy within the scope of the present invention permits better use of the machining tools because of reduced wear, and also makes the formation of material agglomerates on the tools less probable, a problem that can cause productive line arrest in order to replace the deteriorated tools.

In relation to the elements Si, Cr, Zn, according to the present invention, these must be considered as undesirable contaminants, and therefore should be reduced as far as possible according to the possibilities of current foundry production technology. The limits fixed by the present invention can be reasonably obtained in practise, without particular modifications to current productive processes or an increase in production costs.

Therefore, the alloy within the scope of the present invention can be considered as an evolution of the alloy class 3103 according to UNI 9003/3 standards, which, in itself is not suited to the production of "endless" capillary tube.

Even the use of aluminium with a level of commercial purity (for example alloy 1070 previously according to UNI 9001/3, now according to UNI EN 573-3 which has replaced it) has also been revealed as not the best choice for the production of "endless" capillary tube because the workability level of this material "1070" (which is a very pure alloy composed of 99.7% in weight of Al and comprising Si at 0.20% in weight max.; Cu at 0.03% in weight max.; Mg at 0.03% in weight max.; Fe at 0.25% in weight max.; and Mn at 0.03% in weight max.; as well as the inevitable impurities) was demonstrated as being critical and not sufficient to guarantee continuous homogeneous endless capillary tube production according to the present invention. This fact can be explained if it is considered that this material generally offers excellent plastic cold workability levels, but combined with a very low mechanical resistance which creates a decided drop in tool performance caused by accumulated material residue on the tools during machining. The interiors of the capillary tubes realised in this manner also show a high level of machining residue.

On the other hand, the alloy 3103 according to UNI 9003/3 has manganese as the main alligation element and is currently widely used in particularly strict applications such as the automotive industry. Alloy 3103 has a mechanical resistance, in the same physical state, of approximately 50 % more than alloy 1070 and maintains good plastic cold workability characteristics. The problems described for alloy 1070 were also encountered by the inventors of the present Application with the alloy 3103 although at a slightly lesser level. In any case, as demonstrated above, it is important to emphasise the fact that alloy 3103 was not generally suitable for the production of "endless" capillary tubes according to the present invention since the composition interval defined by the standards in question, identifies an alloy family with properties that are too different from one another. If it is considered that for an alloy 3103 the corresponding mechanical characteristics can vary by more than 25 % in terms of mechanical resistance (from 95 to over 120 N/mm2 for an extruded tube, and from approximately 145 to over 185 N/mm2 for a capillary tube not subjected to heat treatment), and since this is only the first step in a succession of further mechanical operations, it would seem that this variability is excessive because it does not permit a production process able to provide constant and repeatable performance with the variations in the composition of the material within acceptable limits.

## Claims

1. Endless capillary tube in aluminium alloy of the type having an internal diameter between the range 0.2 - 4.5 mm and a length within the range 100 - 10000 mm, **characterised in that** the flow rate of two segments of the capillary tube having a length of 2500 mm cut from two positions taken at random from the endless capillary tube does not vary by more than ±6%, wherein the aluminium alloy consisting of: Si 0.15% in weight max., Fe 0.25% in weight max., Cu 0.10% in weight max., Mn 0.90-1.10% in weight max., Mg 0.06% in weight max. ,Cr 0.06% in weight max., Zn 0.10% in weight max., Ti 0.06% in weight max., the remainder being aluminium and inevitable impurities.

2. Endless capillary tube in aluminium alloy according to the first claim **characterised in that** the flow rate of the two segments does not vary by more than ±3%, preferably ±2%, more preferably ±1%.

3. Endless capillary tube in aluminium alloy according to claim 1 or 2, **characterised in that** it is wound to form rolls or wound coils.

4. Method for the production of endless capillary tubes in aluminium alloy as described in the previous claims comprising the following stages:
• Hot extrusion of a roughed blank;
• Successive stages of cold drawing, the number of stages depending on the envisaged machining cycle; the external diameter and the tube thickness are reduced with each extrusion stage until the final measurement is obtained;
• Winding to form wound coils;.
• Washing of the internal surface to eliminate machining residue ;
• Heat treatment to modify the mechanical characteristics of the capillary tube increasing the ductility;

5. Capillary tube in aluminium alloy according to claim 1, **characterised in that** geometrical division in two of the capillary tube produces two equal sections having the same length, and whose respective flow rates do not differ from each other by more than ±6%.

6. Capillary tube according to claim 5 wherein the flow rate of the two halves does not vary by more than ±3%, preferably ±2%, more preferably ±1%.

7. Use of the capillary tube according to claim 5 or 6 to obtain a lamination valve for household appliances.

8. Endless capillary tube in aluminium alloy according to claims 1-3, 5, 6 wherein the aluminium alloy is composed of: Si: 0.10% in weight max.; Fe: 0.20% in weight max.; Cu: 0.10% in weight max.; Mn: 0.90 -1.10% in weight; Mg: 0.03% in weight max.; Cr: 0.03% in weight max.; Zn: 0.07% in weight max.; Ti: 0.03% in weight max.; the remainder being aluminium and inevitable impurities.

9. Endless capillary tube in aluminium alloy according to claims 1-3, 5, 6 wherein the aluminium alloy according is composed of Si: 0.10% in weight max.; Fe: 0.15% in weight max.; Cu: 0.10% in weight max.; Mn: 1.00 - 1.10% in weight; Mg: 0.03% in weight max.; Cr: 0.03% in weight max.; Zn: 0.07% in weight max.; Ti: 0.03% in weight max.; the remainder being aluminium and inevitable impurities.

10. Lamination valve for household appliances comprising a capillary tube according to claims, 1-3, 5, 6, 8, 9.

## Patentansprüche

1. Endloskapillarrohr aus einer Aluminiumlegierung, von dem Typ, der einen Innendurchmesser in dem Bereich zwischen 0,2 und 4,5 mm und eine Länge in dem Bereich von 100 bis 10.000 mm aufweist,
**dadurch gekennzeichnet, dass**
der Durchsatz zweier Segmente des Kapillarrohrs mit einer Länge von 2.500 mm, die an zwei zufällig ausgewählten Positionen aus dem Endloskapillarrohr herausgeschnitten werden, um nicht mehr als ± 6 % variiert, wobei die Aluminiumlegierung besteht aus: maximal 0,15 Gew.-% Si, maximal 0,25 Gew.-% Fe, maximal 0,10 Gew.-% Cu, maximal 0,90 - 1,10 Gew.-% Mn, maximal 0,06 Gew.-% Mg, maximal 0,06 Gew.-% Cr, maximal 0,10 Gew.-% Zn, maximal 0,06 Gew.-% Ti, wobei der Rest aus Aluminium und unvermeidbaren Verunreinigungen besteht.

2. Endloskapillarrohr aus einer Aluminiumlegierung nach Anspruch 1,
**dadurch gekennzeichnet, dass**
der Durchsatz der zwei Segmente um nicht mehr als ± 3 % variiert, vorzugsweise um nicht mehr als ± 2 %, bevorzugter um nicht mehr als ± 1%.

3. Endloskapillarrohr aus einer Aluminiumlegierung nach Anspruch 1 oder 2,
**dadurch gekennzeichnet, dass**
es gewunden ist, um Rollen oder gewundene Spulen zu bilden.

4. Verfahren zur Herstellung von Endloskapillarrohren aus einer Aluminiumlegierung, wie sie in den vorstehenden Ansprüchen beschrieben sind, die folgenden Schritte umfassend:
• Heißstrangpressen eines aufgerauten Rohlings;
• aufeinanderfolgende Stufen des Kaltziehens, wobei die Anzahl der Stufen von dem in Betracht gezogenen Bearbeitungszyklus abhängt; wobei der Außendurchmesser und die Dicke des Rohres mit jeder Stufe des Strangpressens verringert werden, bis der endgültige Messwert erhalten wird;
• Winden, um gewundene Spulen zu bilden;
• Waschen der Innenflächen, um Bearbeitungsreste zu beseitigen;
• Wärmebehandlung zum Modifizieren der mechanischen Eigenschaften des Kapillarrohrs, wodurch die Verformbarkeit erhöht wird.

5. Kapillarrohr aus einer Aluminiumlegierung nach Anspruch 1,
**dadurch gekennzeichnet, dass**
die geometrische Zweiteilung des Kapillarrohrs zwei gleiche Abschnitte mit derselben Länge erzeugt und dass sich deren jeweilige Durchsätze um nicht mehr als ± 6 % voneinander unterscheiden.

6. Kapillarrohr nach Anspruch 5,
wobei der Durchsatz der zwei Hälften um nicht mehr als ± 3 % variiert, bevorzugt um nicht mehr als ± 2 %, bevorzugter um nicht mehr als ± 1 %.

7. Verwendung des Kapillarrohrs nach Anspruch 5 oder 6,
um ein Beschichtungsventil für Haushaltsanwendungen zu erhalten.

8. Endloskapillarrohr aus einer Aluminiumlegierung nach Anspruch 1. bis 3, 5, 6,
wobei die Aluminiumlegierung besteht aus: Si: maximal 0,10 Gew.-%; Fe: maximal 0,20 Gew.-%; Cu: maximal 0,10 Gew.-%; Mn: 0,90-1,10 Gew.-%; Mg: maximal 0,03 Ges.-%; Cr: maximal 0,03 Gew.-%; Zn: maximal 0,07 Gew.-%; Ti: maximal 0,03 Gew.-%; wobei der Rest aus Aluminium und unvermeidbaren Verunreinigungen besteht.

9. Endloskapillarrohr aus einer Aluminiumlegierung nach Anspruch 1 bis 3, 5, 6,
wobei die Aluminiumlegierung besteht aus: Si: maximal 0,10 Gew.-%; Fe: maximal 0,15 Gew.-%; Cu: maximal 0,10 Gew.-%; Mn: 1,0 - 1,1 Gew.-%; Mg: maximal 0,03 Gew.-%; Cr: maximal 0,03 Gew.-%; Zn: maximal 0,07 Gew.-%; Ti: maximal 0,03 Gew.-%; wobei der Rest aus Aluminium und unvermeidbaren Verunreinigungen besteht.

10. Beschichtungsventil für Haushaltsanwendungen, das ein Kapillarrohr nach Anspruch 1 bis 3, 5, 6, 8, 9 umfasst.

## Revendications

1. Tube capillaire sans fin en alliage d'aluminium du type ayant un diamètre interne compris dans la plage de 0,2 à 4,5 mm et une longueur dans la plage de 100 à 10 000 mm, **caractérisé en ce que** le débit de deux segments du tube capillaire ayant une longueur de 2 500 mm découpée à partir de deux positions prises au hasard du tube capillaire sans fin ne varie pas de plus de ± 6%, dans lequel l'alliage d'aluminium consiste en : 0,15% en poids max. de Si, 0,25 % en poids max. de Fe, 0,1.0 % en poids max. de Cu, 0,90 à 1,10% en poids max. de Mn, 0,06 % en poids max. de Mg, 0,06% en poids max. de Cr, 0,10 % en poids max. de Zn, 0,06 % en poids max. de Ti, le reste étant constitué d'aluminium et d'impuretés inévitables.

2. Tube capillaire sans fin en alliage d'aluminium selon la première revendication, **caractérisé en ce que** le débit des deux segments ne varie pas de plus de ± 3 %, de préférence de ± 2 %, de manière davantage préférée de ± 1 %.

3. Tube capillaire sans fin en alliage d'aluminium selon la revendication 1 ou 2, **caractérisé en ce qu'**il est enroulé pour former des rouleaux ou des bobines enroulées.

4. Procédé de production de tubes capillaires sans fin en alliage d'aluminium tels que décrits dans les revendications précédentes, comprenant les étapes suivantes :
- l'extrusion à chaud d'une ébauche dégrossie ;
- des étapes successives d'étirage à froid, le nombre d'étapes dépendant du cycle d'usinage envisagé ; le diamètre externe et l'épaisseur du tube sont réduits avec chaque étape d'extrusion jusqu'à l'obtention de la mesure finale ;
- l'enroulement pour former des bobines enroulées ;
- le lavage de la surface interne pour éliminer les résidus d'usinage ;
- le traitement par la chaleur pour modifier les caractéristiques mécaniques du tube capillaire en augmentant la ductilité.

5. Tube capillaire en alliage d'aluminium selon la revendication 1, **caractérisé en ce que** la division géométrique en deux du tube capillaire produit deux sections égales ayant la même longueur, et dont les débits respectifs ne diffèrent pas l'un de l'autre de plus de ± 6 %.

6. Tube capillaire selon la revendication 5,dans lequel le débit des deux moitiés ne varie pas de plus de ± 3 %, de préférence ± 2 %, de manière davantage préférée ± 1 %.

7. utilisation du tube capillaire selon la revendication 5 ou 6, pour obtenir une valve de laminage destinée à des appareils électroménagers.

8. Tube capillaire sans fin en alliage d'aluminium selon les revendications 1 à 3, 5 et 6, dans lequel l'alliage d'aluminium est composé : de 0,10 % en poids max. de Si ; de 0,20 % en poids max. de Fe ; de 0,10 % en poids max. de Cu, de 0,90 à 1,10% en poids max. de Mn ; de 0,03 % en poids max. de Mg ; de 0,03 % en poids max. de Cr ; de 0,07% en poids max. de Zn ; de 0,03 % en poids max. de Ti, le reste étant constitué d'aluminium et d'impuretés inévitables.

9. Tube capillaire sans fin en alliage d'aluminium selon les revendications 1 à 3, 5 et 6, dans lequel l'alliage d'aluminium est composé : de 0,10% en poids max. de Si ; de 0,15% en poids max. de Fe ; de 0,10 % en poids max. de Cu ; de 1,00 à 1,10 % en poids max. de Mn ; de 0,03 % en poids max. de Mg ; de 0,03 % en poids max. de Cr ; de 0,07% en poids max. de Zn ; de 0,03 % en poids max. de Ti, le reste étant constitué d'aluminium et d'impuretés inévitables.

10. Valve de laminage destinée à des appareils électroménagers comprenant un tube capillaire selon les revendications 1 à 3, 5, 6, 8 et 9.
